

- [54] OIL RECOVERY METHOD FOR  
DISPLACEMENT ROTARY AIR  
COMPRESSOR
- [75] Inventor: Eiichi Uratani, Tokyo, Japan
- [73] Assignee: Sumida Equipment Industries, Inc.,  
Tokyo, Japan
- [22] Filed: Sept. 1, 1972
- [21] Appl. No.: 285,872

- [30] Foreign Application Priority Data  
Mar. 29, 1972 Japan ..... 47-30686
- [52] U.S. Cl. ..... 55/29
- [51] Int. Cl. ..... B01d 53/14
- [58] Field of Search ..... 55/45, 29, 34, 32; 210/21,  
210/22, 168; 252/58, 59
- [56] References Cited  
UNITED STATES PATENTS
- 3,363,399 1/1968 Schmauch et al. ..... 55/45  
3,564,863 2/1971 Sasseui ..... 210/168

3,634,247 1/1972 Parker ..... 252/58

OTHER PUBLICATIONS

"Effects of Refrigerants on Lubricating Oils" Lubrication, Vol. 47, No. 7, Texaco, Inc., July 1961, pp. 78-80.

Primary Examiner—Charles N. Hart  
Attorney, Agent, or Firm—Hans Berman

[57] ABSTRACT

The turbine oil used in a screw-type air compressor as a lubricant and sealant is mixed with approximately 40 percent trichlorofluoromethane, trichlorotrifluoroethane, or dichlorotetrafluoroethane to raise the specific gravity of the mixture above that of water. When the compressed air discharged from the compressor is cooled, moisture condenses and the entrained droplets of the oil mixture are precipitated and settle under the aqueous condensate so that the latter may be removed by overflow while the oil mixture may be returned to the compressor.

7 Claims, 2 Drawing Figures



PATENTED JUN 4 1974

3,813,850

*Fig. 1*



*Fig. 2*



## OIL RECOVERY METHOD FOR DISPLACEMENT ROTARY AIR COMPRESSOR

This invention relates to an oil recovery method for an air compressor, and more particularly, to a method of recovering oil used in the lubrication, cooling, and sealing of positive displacement rotary air compressors such as a screw type compressor or the like.

Generally, the removal of oil from compressed air and dehydration thereof is required before the use of such compressed air since the compressed air discharged or exhausted from the compressor contains the compressor lubricating oil and water therein. The currently and widely available screw type compressor uses much oil for lubrication, cooling, and sealing thereby leaving much oil in the exhausted air. For this reason, the problem of oil separation (or oil recovery) has been critical. In the conventional screw type compressor, it has been the practice heretofore that the air exhausted from the compressor is led to the oil separator (or oil recovering device) in which the oil is separated from the air, and then the separated and recovered oil as it is or cooled is returned to the compressor. However, this does not satisfactorily remove all the oil from the air and the quality of compressed air is impaired for all the outstanding functions of the screw type compressor. The compressed air thus obtained is restricted in use and the compressor requires much consumption of oil. The oil recovered and reused contains moisture which rusts the compressor. In addition, the compressor is not cooled sufficiently.

More specifically, anti-emulsifying oil is conventionally used in the screw type compressor so that the oil finely divided as a mist is carried in the exhausted air separately from the water. This allows the oil to readily pass along with the air through the oil separator. In fact, it has been found that capture of oil in the oil separator is complete if the exhausted air is cooled to form the finely divided oil into relatively large droplets. However, this increases the condensation of water. Cooling of the compressor is also accompanied by an increase in the condensation of water. Water of condensation has a higher specific gravity than that of oil and may lay under the layer of oil in the oil separator to rust the compressor if this condensed water is fed along with the air to the compressor and should the quantity of condensed water become large, it may lead to burning out of the compressor due to poor lubrication. In this connection, separation of water from the oil and disposition of the water are necessary, but it is very difficult to automatically discharge the water from under the oil. Thus the prior art apparently has failed to not only lower the temperature of compressed air to be treated by the oil separator to an extent suitable for oil separation but also to cool down the compressor sufficiently.

Accordingly, it is an object of the present invention to provide a method of recovering oil from the compressed air which allows both to lower the temperature of the compressor, oil and the exhausted compressed air sufficiently for protection of the compressor and removal of oil and also to completely separate the condensed water from the recovered oil and dispose of the water whereby eliminating difficulty in re-use of the recovered oil.

According to the invention, this object is accomplished by adding and mixing a proper material with the

oil to be used to cause the oil to reach a higher specific gravity than that of water.

More particularly, when an additive material is mixed with the oil for lubrication of the compressor or for other purposes it properly increases the specific gravity of oil to more than that of water thereby reversing the normal specific gravity relationship between water and oil. Thus, in the oil separator the condensed water is supernatant over, and distinctly separated from, the recovered oil (normally the water is deposited below the layer of oil). As a result, the condensed water is readily and completely separated from the oil and disposed of by automatically over-flowing the water. This prevents the water from being mixed with the recovered oil to be reused so that the condensation of water makes no interference with the recovery of oil. This enables the compressor, oil and the exhausted compressed air to be cooled sufficiently enough for protection of the compressor and removal of oil.

The complete cooling of the compressor and removal of oil (or oil recovery) above referred to increases the life-time of the compressor and makes it less costly to maintain the same and reduces the consumption of oil and avoids acid deterioration of oil.

It should be noted that the method in accordance with the invention can be carried out with utilizing the conventional installation and arrangement almost without modifying them.

FIG. 1 is a schematic representation showing a typical oil recovery apparatus system for the compressor in which the conventional method is carried out, and

FIG. 2 is a schematic representation showing a preferred oil recovery apparatus system for the compressor in which a method according to the present invention is carried out.

Preferred properties of the aforementioned additive material are as follows:

1. The boiling point of additive material under atmospheric pressure is higher than the freezing point of water but lower than the boiling point thereof. (The additive material should not be evaporated within the compressed air.)
2. The solubility of additive material is high with respect to the oil but is low with respect to the water (for the purpose of adding to the oil to be used and of facilitating its separation from the condensed water.)
3. The additive material should be of high specific gravity (for the purpose of adding to the oil to be used thereby causing the specific gravity of oil to be more than that of water.)
4. The additive material must have appropriate viscosity (to provide the oil with appropriate lubricant property.)
5. The additive material should be noninflammable, non-toxic, and anti-corrosive to machinery and tools.

The following compounds have been found to be suitable in carrying out the invention as a result of various experiments in view of the aforementioned preferred properties of additive material.

| Identification as Refrigerant | Chemical Formula                              | Name of Compound         |
|-------------------------------|-----------------------------------------------|--------------------------|
| R-11                          | CCl <sub>3</sub> F                            | Trichlorofluoromethane   |
| R-113                         | C <sub>2</sub> Cl <sub>3</sub> F <sub>3</sub> | Trichlorotrifluoroethane |

R-114

 $C_2Cl_2F_4$ 

Dichlorotetrafluoroethane

Preferred addition rates of these additive materials to the oil in volume percent of the oil before mixing are as follows. The oil which has the additive material mixed at such rate, provides kinetic viscosity of 11-15-cst/30°C and specific gravity of 1.1kg/1.

Additive Oil in Use (turbine oil according to Japanese Industrial Standard)

|       | No. 200 | No. 180 | No. 140 |
|-------|---------|---------|---------|
| R-11  | 38-42   | 38-40   | —       |
| R-113 | 40-45   | 38-42   | 34-37   |
| R-114 | 39-41   | —       | —       |

These oils having additive material added as above exhibit performances similar to that of conventional oils in lubrication, cooling, and sealing for the compressor.

A preferred arrangement for carrying out the invention will be hereinafter explained by reference to the accompanying drawing.

In FIG. 1, there is shown conventional oil recovery systems, wherein conventional oil fed to a screw type air compressor 1 serves for lubrication, cooling, and sealing in the compressor and passes through a check valve 2 and then into an oil separator (or oil recovery device) 3 together with the compressed air. The oil separated and recovered from the air by the oil separator passes through an oil temperature regulating valve or an oil cooler 4 and is again fed back to the compressor by an oil pump 6.

It is noted that in the prior art systems the compressed air containing oil is not cooled yet before passing through the oil separator (to prevent the water from being condensed by cooling, as above mentioned).

The condensed water deposited in the bottom of the oil separator can be drained through a drain valve 7.

As above mentioned, it is impossible to automatically discharge the condensed water from the oil separator since the conventional oil has a lower specific gravity than water to allow the water to be deposited below the layer of oil.

Referring to FIG. 2, there is illustrated a typical system with which the present invention is carried out. The additive material is mixed with the oil to be supplied into the screw type air compressor 1 whereby the oil exhibits a heavier specific gravity than that of water. The oil having the additive material mixed, serves for lubrication, cooling and sealing in the compressor in the same manner as the conventional oil and is discharged with the compressed air through the check valve 2. The compressed air with oil is fully cooled in a cooler 4 before the oil separator (or recovery device) 3. This differs from the prior art system shown in FIG. 1, as precisely mentioned hereinbefore. The condensed water and oil are separated from the compressed air by the oil separator and then distinctly divided into two phases, wherein the oil is deposited below the layer of

water in the oil separator. The oil thus recovered is again fed back to the compressor by the oil pump 6 whereas the supernatant water automatically overflows and is discharged through an auto-drain valve (or overflow discharge valve) 7'.

The invention has been described in detail with particular reference to preferred embodiments thereof, but it will be understood that variations and modifications can be effected within the spirit and scope of the invention.

What I claim is:

1. In a method of operating an air compressor in which lubricating oil having a specific gravity lower than that of water is supplied to the compressor, moisture and entrained oil droplets are discharged from said compressor with the compressed air and are removed from said air by cooling said air until moisture is condensed and entrained oil droplets are precipitated from said air, and the precipitated oil and condensed moisture are separated by settling, the improvement which comprises mixing said oil prior to said discharging with an amount of an additive having a boiling point at atmospheric pressure higher than the freezing point of water and lower than the boiling point of water, said additive being more soluble in said oil than in said water, having a specific gravity sufficiently higher than that of said water to raise the specific gravity of the mixture of said oil with said amount of additive above that of water, and a viscosity sufficient to substantially maintain the lubricant properties of said oil when added to the same in said amount, said additive being non-corrosive to machinery and tools, whereby said condensed moisture forms a supernatant on the precipitated mixture after said cooling.

2. In a method as set forth in claim 1, said additive being trichlorofluoromethane, trichlorotrifluoroethane, or dichlorotetrafluoroethane.

3. In a method as set forth in claim 1, said additive being trichlorofluoromethane, and being added to said lubricating oil in an amount of 38 percent to 42 percent of the volume of said oil.

4. In a method as set forth in claim 1, said additive being trichlorotrifluoroethane, and being added to said lubricating oil in an amount of 34 percent to 45 percent of the volume of said oil.

5. In a method as set forth in claim 1, said additive being dichlorotetrafluoroethane, and being added to said lubricating oil in an amount of 39 percent to 41 percent of the volume of said oil.

6. In a method as set forth in claim 1, separating said supernatant condensed moisture from said mixture by overflowing said moisture, and returning said mixture to said compressor.

7. A method as set forth in claim 1, wherein said additive is added to said lubricating oil before said lubricating oil is supplied to said compressor.

\* \* \* \* \*